

# UNITED STATES PATENT OFFICE.

AUGUSTE J. ROSSI, OF NIAGARA FALLS, NEW YORK, ASSIGNOR TO THE TITANIUM ALLOY MANUFACTURING COMPANY, OF NEW YORK, N. Y., A CORPORATION OF MAINE.

ARTICLE COMPOSED ESSENTIALLY OF TITANIUM AND SILVER AND METHOD OF PRODUCING THE SAME.

1,024,476.

Specification of Letters Patent. Patented Apr. 23, 1912.

No Drawing.

Application filed January 30, 1912. Serial No. 674,257.

*To all whom it may concern:*

Be it known that I, AUGUSTE J. Rossi, a citizen of the United States, and a resident of Niagara Falls, in the county of 5 Niagara and State of New York, have invented a certain new and useful Article Composed Essentially of Titanium and Silver and Methods of Producing the Same, of which the following is a specification.

10 The objects of my present invention comprise the production of a binary alloy of titanium with silver and provision of methods for producing it, so simple and reliable in operation, and so economical, as 15 to justify manufacture on industrial scales. I attain these objects as hereinafter described. I have discovered that the said binary alloy of titanium with silver is exceptionally useful for the purpose of purifying silver in mass as heretofore produced 20 in the usual processes of manufacture. Silver, while in molten state, absorbs gaseous elements or compounds, which are dissolved in the metal and retained therein as it 25 solidifies during cooling. For instance oxygen from the atmosphere is thus very largely absorbed, and, to a great extent, combined chemically with the silver, forming oxids thereof, which, together with 30 oxygen, if any, remaining uncombined, are found occluded in the mass of the solidified metal. The aforesaid foreign elements and compounds are usually unhomogeneously distributed in uncontrollable locations 35 throughout the mass of the metal, thus producing blow-holes or other cavities or pits on the surface. The presence of such impurities and their resultant imperfections in the metal not only disfigure 40 it for certain purposes for which a high and perfect polished surface is desired, but also, after solidification of the metal, tend to subsequent additional deteriorations of the metal, including particularly its continued undesirable oxidation by normal 45 outside influences. The impurities mentioned, and their results on the metal, depreciate its value in mass for many special purposes, as will be readily understood. I 50 have discovered that the said undesirable impurities can all of them be eliminated by adding to the silver, while molten, metallic titanium in amounts proportioned to

satisfy the chemical affinities therefor of such undesired elements and compounds 55 and also properties desirable in some cases imparted by increasing such amount so as to retain in the resulting product a moderate proportion as for instance less than one per cent. of titanium. 60

Segregated titanium is still I believe unattainable in quantities sufficient for operations on an industrial scale or at all events unattainable except at too great cost. Moreover the peculiar characteristic properties of titanium, as compared with those 65 of silver, cause it to less well and readily incorporate therewith when added thereto by itself alone than when added thereto in the form of an alloy thereof with silver. 70 My hereinafter described novel alloy of titanium and silver is therefore of particular importance and utility for the purpose of purifying silver, or imparting thereto novel properties as aforesaid, as well as for 75 other uses.

I prefer to produce my said novel alloy of titanium and silver as follows:—I first charge into a graphite crucible, or other container properly adapted, some silver 80 sufficient on being melted to form a small supporting or initiatory bath of that metal. To such silver I add an oxid of silver, for instance  $Ag_2O$ , and also titanic acid mixed therewith in such proportions as, on reduction, taken together with the silver of the bath, to impart to the resulting alloy the desired respective proportions of the two metals. To the said silver and mixture of 85 oxids I also add such an amount of aluminum (preferably in shots or the like so as to melt more rapidly) as is chemically sufficient to decompose the oxids of silver and of titanium and reduce their respective titanium and silver contents to their metallic 90 states. This mixture is then heated by any convenient means to a point at which the aluminum melts, thereby supplying a bath of molten aluminum to the charge. The additional heat developed by the reduction 95 of the oxid of silver by the aluminum rapidly raises the charge to a temperature required to set up the reduction of the oxid of titanium by the aluminum, which then proceeds until the reduction of all the 100 oxids present is completed. Care should be 105

taken at this point to maintain the temperature of the charge sufficiently high, as by an electric furnace for instance, to maintain the fluidity of the nascent alloy, the 5 reactions to which the latter is due being as per the following formulæ, assuming that  $\text{Ag}_2\text{O}$  is the oxid of silver employed:—



I prefer to employ the foregoing method largely because of its economy, the cost of the oxid requisite to produce the required amount of silver being considerably less than 10 that of such amount of silver in metallic form, and also because the heat of formation of oxid of silver is so small compared to that of the formation of aluminum oxid as to leave a large surplus of heat immediately 15 applicable to the reduction of the oxid of titanium whereby the reactions are promoted and accomplished at a considerably less expenditure of external heat than required where silver altogether is alone employed in the charge. It will be understood, 20 however, that the said alloy may be produced, though not so advantageously, by substantially the process above referred to by using as the argentic material in the 25 process above referred to metallic silver exclusively, or, on the other hand, by using as such argentic material oxid of silver exclusively. The molten product on being withdrawn and cooled will be found to be an 30 alloy of titanium and silver, the percentage of the former being proportional to the amounts of titanium oxid and aluminum charged.

My said alloy of titanium and silver may 35 also, though not so advantageously, be produced by substituting carbon for aluminum as the reducing agent, in which case it is essential, in industrial practice, to employ such high temperatures as are derivable from 40 some of the now well known forms of electric furnaces, such for example as illustrated and described in Letters Patent No. 802,941, granted to me October 24, 1905. In this case, 45 oxid of silver, oxid of titanium, and carbon 50 are employed as per the formulæ:—



The said ingredients, either with or without 55 some metallic silver as may be preferred,

are changed in said furnace and the current turned on. This will result in production of a bath of molten silver, and the current being continued the titanium oxid will be reduced to titanium which mingles or dissolves in 60 said bath of silver to constitute the said alloy. In this instance, like the foregoing, the addition of silver in metallic state, though not absolutely necessary, facilitates the reduction of the titanium oxid by the carbon 65 and it will of course be understood that the alloy may be thus produced by using as the only argentic material of the charge metallic silver.

The proportions of the ingredients used 70 in the charge will be varied according to the percentage of the respective metals desired in the alloy according to the formulas above given and as experience and test in each case will readily demonstrate to those skilled in 75 the metallurgical art is required for the particular purpose for which the alloy is to be used.

What I claim as new and desire to secure by Letters Patent is the following, viz:— 80

1. As a new article an alloy of titanium with silver.

2. The method of producing an alloy of titanium with silver which comprises incorporating titanic acid into a bath of molten 85 silver in presence of a reducing agent, subjecting the bath to a temperature sufficient to insure reduction of said titanic acid by said agent, and withdrawing and cooling the resulting metallic product. 90

3. The method of producing an alloy of titanium with silver which comprises bringing together argentic material, titanic acid and carbon, and subjecting the combination to a temperature sufficient to insure production therefrom of molten silver and molten 95 aluminum. 95

4. The method of producing an alloy of titanium with silver which comprises bringing together oxid of silver, oxid of titanium 100 and carbon, and subjecting the combination to a temperature sufficient to insure reduction of said oxid by said carbon and then withdrawing and cooling the resulting metallic product.

AUGUSTE J. ROSSI.

Witnesses:

WALTER D. EDMONDS,  
PHILIP C. PECK.